

# UNITED STATES PATENT OFFICE.

RENÉ BOHN, OF MANNHEIM, GERMANY, ASSIGNOR TO BADISCHE ANILIN & SODA FABRIK, OF LUDWIGSHAFEN-ON-THE-RHINE, GERMANY, A CORPORATION.

## PROCESS OF BUCKING VEGETABLE MATERIAL.

1,156,048.

Specification of Letters Patent. Patented Oct. 12, 1915.

No Drawing. Original application filed January 27, 1909, Serial No. 474,485. Divided and this application filed November 6, 1913. Serial No. 793,484.

To all whom it may concern:

Be it known that I, RENÉ BOHN, Ph. D., citizen of the Swiss Republic, residing at Mannheim, Germany, have invented new and useful Improvements in the Process of Bucking Vegetable Material, of which the following is a specification.

This application is a division of my original application Serial No. 474,485, filed January 27, 1909, and relates to a process of bucking.

Few, if any, coloring matters, when dyed or printed on vegetable fiber, are perfectly fast against bucking (that is, heating for a considerable time with dilute caustic alkali solution), particularly when the bucking is carried out under pressure. Attempts have been made to avoid this disadvantage of bucking by adding an inorganic oxidizing agent, such for instance as sodium bichromate and potassium permanganate, to the bath used. These, however, are not satisfactory because, when bichromate is used, the chromium oxid which is formed colors the material yellow, and also when permanganate is used, the material is stained and the removal of such stains is a complicated process and tends to weaken the fiber.

I have now discovered that vegetable material dyed or printed with vat coloring matter can be successfully bucked without the color passing into the white or spreading beyond its proper limits, if the bucking vat contain dilute alkali solution and an organic compound which is soluble and easily reducible in the presence of alkali. The alkali used may be caustic or carbonate or a salt possessing an alkaline reaction, like sodium phosphate or borax, or again mixtures of these alkalis can be used. As examples of suitable soluble and easily reducible organic compounds I mention anthraquinone derivatives and nitro derivatives,

and in particular salts of anthraquinone sulfonic acid, anthraquinone disulfonic acid, nitrobenzene sulfonic acid, and nitro-toluene sulfonic acid.

In order to prepare a bucking vat I take, for instance, the following ingredients in approximately the proportions indicated, namely 4,000 parts of water, 13 parts of solid caustic soda and 8 parts of the sodium salt of nitrobenzene sulfonic acid, or instead of 8 parts of the sodium salt of nitrobenzene sulfonic acid the same quantity of the sodium salt of anthraquinone monosulfonic acid or anthraquinone disulfonic acid can be used. The material to be bucked is introduced into this bath and boiled for about 2 hours at a pressure of 2 atmospheres in excess of ordinary pressure.

Now what I claim is:

1. The process of bucking vegetable material dyed or printed with vat coloring matter, by heating the said material with a dilute alkali solution in the presence of an organic compound which is soluble and easily reducible in the presence of alkali.

2. The process of bucking vegetable material dyed or printed with vat coloring matter, by heating the said material with a dilute caustic soda solution in the presence of a salt of nitrobenzene-sulfonic acid.

3. The process of bucking vegetable material dyed or printed with vat coloring matter, by heating the said material with a dilute caustic soda solution in the presence of the sodium salt of nitrobenzene-monosulfonic acid.

In testimony whereof I have hereunto set my hand in the presence of two subscribing witnesses.

RENÉ BOHN.

Witnesses:

J. ALEC. LLOYD,  
S. S. BERGER.